

## UNITED STATES PATENT OFFICE

2,606,188

OXIDIZED STARCH AND METHOD OF  
PREPARING THE SAMEWilliam E. C. Yelland, Washington, D. C., assignor  
to Lauhoff Grain Company, Danville, Ill., a cor-  
poration of IllinoisNo Drawing. Application August 2, 1949,  
Serial No. 108,227

5 Claims. (Cl. 260—233.3)

## 1

This invention relates to modified starch and more particularly to starch that has been oxidized with periodic acid to modify the molecular structure thereof and to produce a product having new and valuable properties and being useful for a variety of purposes, especially for the warp sizing of textile yarns. The invention also relates to a process for preparing modified starch by the oxidation of starch with periodic acid under controlled conditions, as set forth more fully hereinafter.

Textile yarns are sized prior to weaving for the purpose of protecting them from abrasion during the weaving operation. Warp sizing also increases the strength of yarns. This increase in strength is most noticeable with low twist yarns and less evident with more highly twisted yarns and continuous filament rayons. Improvement in these properties results in increased weave room efficiency and better fabric quality. In the case of comparatively rough, fuzzy yarns, such as cotton and spun rayon, rather viscous sizes are used to produce a heavy coating of size on the outside of the yarn, with sufficient penetration of the size into the interior of the yarn to anchor the size film firmly to the yarn. This film ties in the fiber ends and thus changes a fuzzy yarn into a relatively smooth one. Consequently, fewer fibers are broken off by abrasion against the loom parts during weaving and there is less "shedding" in the loom. Thus an increase in weave room production is achieved. In the case of smooth yarns, such as continuous filament rayon yarn, less viscous size mixes are used. These tend to produce thin, flexible films of size on the yarn which prevent broken filaments from sliding back along the yarn during weaving and producing "fuzz-balls" or "birds' nests," which eventually entangle adjacent yarns and cause end breakage.

In addition to protecting the yarn during weaving, the size must be capable of being removed, prior to dyeing, without damage to the fabric. Unmodified commercial starches, such as thick-boiling corn starch, are not readily desized after weaving. This has led to the development of thin-boiling starches, British gums, and dextrins. Thin-boiling starches are used primarily on cottons, and are essentially products obtained by acid hydrolysis of starch in the form of a wet slurry. British gums are used extensively on spun rayon and are produced usually by roasting starch (i. e. heating it in the dry state, with only its natural moisture content) in the presence of traces of alkali. Dextrins are made by roasting starch in the presence of catalysts and/or traces of acids.

## 2

While the foregoing materials are somewhat more readily desized from the fabric than raw starch they still usually require treatment with enzymes for satisfactorily complete removal.

5 Also the thin-boiling starches have the disadvantage that, since they are made by a hydrolytic process, increased solubility is obtained by shortening the main carbohydrate chain in the starch molecule. This leads to materials 10 which have lower film strength and greater brittleness and, consequently, are of less value in warp sizing. Although the mechanisms of gum and dextrin formation are not completely understood, it is a well known fact that highly converted materials of this sort have undergone considerable molecular degradation and their films are weaker and more brittle than those of the original unmodified starch.

An object of the invention is to provide a 20 modified starch that is especially suitable for warp sizing of textile yarns and other sizing operations.

Another object is to provide a modified or 25 oxidized starch that has film-forming and adhesive properties similar to those of unmodified starch but that exhibits a much greater ability to be dissolved or dispersed in dilute solutions of alkali.

Another object is to provide a modified starch 30 for warp sizing and like uses that may be removed from the fabric, after weaving, with a mild alkaline scour and without the use of enzymatic desizing preparations.

Another object of the invention is to provide 35 a process for the modification or oxidation of starch utilizing periodic acid as the oxidizing agent.

The modified starches of the invention may 40 be prepared from a wide variety of unmodified or partially modified starches. The following starting materials may be employed: raw corn starch, Amioca starch which is a type of corn starch consisting mainly of the branched chain fraction and substantially free from amylose, 45 wheat starch, tapioca starch, potato starch, sago starch, thin-boiling (i. e. acid-hydrolysed) starch, corn starches already modified to some extent with alkaline hypochlorite, and crude corn starches containing up to 3.5% of protein and some oil.

The modified starches of the invention are 50 characterized by many properties similar to those of the unmodified starting materials. Among these are: (1) a general or superficial appearance to the naked or unaided eye substantially identical to or strongly resembling the unmodified starting material; (2) a grain struc-

ture as viewed under the microscope similar to that of the untreated starting material; (3) the showing of a polarization cross under polarized light that is typical of the cross exhibited by the starting material; (4) a substantial retention of the highly polymeric structure of the unmodified starch; (5) the characteristic that pastes formed of the modified starch at normal pH (5 to 7 approximately) are substantially as viscous as those formed from the original starch and the film-forming properties and film characteristics such as flexibility, tensile strength and like physical properties are not substantially diminished in the products of the invention.

The modified starches of the invention have other properties that differ markedly from the corresponding properties of the starting materials. For example, alkaline solutions dissolve or disperse the modified starches to a much greater extent and much more rapidly than they do the starting materials.

Although the invention is not dependent on the correctness of any theory, it is believed that the molecular structure of the starch is changed by reaction of the periodic acid with a substantial number of the anhydroglucose units of the starch probably essentially as follows:



The conversion of two adjacent hydroxyl groups into aldehyde groups, although it opens the ring, does not break the main carbohydrate chain. However, opening the ring makes the compound especially sensitive to alkali so that treatment, even with mild alkali, tends to break the chain at the carbon atoms once removed from the opening in the ring. Thus are produced starch derivatives, which at their normal pH values, (pH 5 to 7 approximately) are good film-forming materials. But the films, once formed, are readily dispersible or even soluble in alkali.

Additionally, the modified starches of the invention show greatly increased alkaline fluidity numbers and much decreased alkaline paste viscosities as compared with the starting materials.

Typically, the process of the invention includes suspending starch in an aqueous liquid and adding thereto periodic acid in an amount based on the dry weight of the starch ranging from about 0.05% to about 0.5% by weight calculated as  $\text{HIO}_4 \cdot 2\text{H}_2\text{O}$ , and maintaining said periodic acid in contact with the starch at a pH of from about 4.5 to about 7.0 at a temperature and for a time sufficient to substantially completely react the periodic acid with the starch. Thereafter, the modified starch is preferably washed and dried. Particularly in the range of from about 0.1% to about 0.35% periodic acid, the resulting oxidized

starches exhibit excellent film-forming properties and greatly improved alkali resolubility or redispersibility.

In carrying out the process of the invention, starch is slurried in water preferably at a concentration of approximately one pound per gallon of water. The starch concentration is not critical and either more concentrated or more dilute slurries can be used. The only limitation is convenience in handling the mixture. If too concentrated a slurry is used it becomes difficult to stir the slurry sufficiently vigorously to insure uniform mixing when the periodic acid solution is added. If too dilute slurries are used, dewatering of the starch after the reaction is complete involves the removal of larger volumes of water than necessary. The concentration of one pound of starch per gallon of water is convenient, but any concentration which can be handled satisfactorily is feasible.

The pH of the slurry is measured and, if necessary, adjusted to a value within the range pH 4.5 to pH 7.0. A preferred working range is pH 4.5 to pH 6.0. Buffered acidic or basic solution may be used to adjust the pH to the desired value. The preferred pH range is close to that of commercial corn starch, that is, approximately pH 5.0, but somewhat higher or lower values can be used. It is inadvisable to work at a pH lower than about 4.5 because the starch molecule may be attacked hydrolytically by the acid rather than being oxidized. It is not advantageous to work above about pH 7.0 because of the comparatively slow reaction rate and the low solubility of peridote salts.

Periodic acid is next added to the slurry, preferably in the form of a dilute aqueous solution and vigorous stirring is maintained so that the starch does not settle out of the slurry. Periodic acid is conveniently obtained as the dihydrate under the name of paraperiodic acid



The acid is in the form of deliquescent crystals and is therefore difficult to weigh accurately. In order to obviate this difficulty, solutions approximately 0.05 molal (11.4 g.  $\text{HIO}_4 \cdot 2\text{H}_2\text{O}$  per liter of solution) are prepared and standardized. The amount of acid required for each preparation is then obtained by measuring out the corresponding volume of solution.

The concentration of the added periodic acid solution is not critical, the more dilute the solution the greater the ease of thorough mixing of the reagent with the starch and the more uniform the product. However, solutions as concentrated as 0.5 molal (114 g.  $\text{HIO}_4 \cdot 2\text{H}_2\text{O}$  per liter of solution) may be used successfully. Solutions of concentrations lower than 0.05 molal can also be used.

The addition of the periodic acid solution may cause a slight lowering of the pH of the slurry.

The reaction is conveniently carried out at ordinary room temperatures of from about 15° C. to about 35° C., but the reaction proceeds well at temperatures as low as about 5° C. to as high as about 80° C. The temperature, however, is not critical and temperatures above and below these limits may be used. In general, the higher the temperature, the more rapid the reaction rate.

Samples of the slurry undergoing reaction are withdrawn at intervals of approximately five minutes each and are tested for periodic acid in conventional manner.

When the test for periodic acid is no longer

positive the reaction is substantially complete. At the concentrations of hydrogen ion used and at room temperature, approximately 15° C.-35° C., the periodic acid reacts very rapidly with the starch. The periodic acid usually reacts completely with the starch in less than ten minutes, and no positive tests for periodic acid are obtained after this time. However, to insure complete reaction, the slurry is stirred for approximately 10 minutes after it shows a negative periodic acid test and then the modified starch is dewatered in any desired or conventional way, as by filtering.

The modified starch filter cake may be washed thoroughly in water to free it substantially from iodic acid as indicated by conventional testing procedures.

If the test for iodic acid is positive, the whole filter cake is reslurried in water, stirred vigorously for five minutes and then filtered a second time. This process is repeated until the filter cake is practically free from iodic acid.

The filter cake is then broken up and dried by any of the conventional means such as are used on raw or unmodified starch. The drying temperature and time should not be such that the moist starch is gelatinized or the dry starch dextrinized. Air drying for at least 24 to 48 hours has been found satisfactory and convenient.

The lumps of dry starch are then pulverized and screened. Unless the degree of modification is excessively high the lumps are found to powder readily and can be easily screened through a 100-mesh screen.

It will be obvious from the foregoing that by varying the amount of acid used in relation to a fixed amount of starch a series of modified starches can be prepared from any raw starch. These will differ mainly in their sensitivity to alkali, the more highly modified starches being more sensitive to alkali and their films being soluble or dispersible at lower pH's and lower temperatures; the less highly modified materials will be less sensitive to alkali and their films will require higher pH's and temperatures to dissolve or disperse them. Since the ease of desizing is a function of the film solubility, it is seen that starches can be prepared with different desizing properties. Consequently, products which can be desized under mild conditions—very dilute alkali and low temperature—can be prepared for use as rayon sizes. For cottons, which can stand more drastic desizing treatment, less readily removable products can be prepared. It then becomes a question of measuring the degree of modification and relating it to the requirements of desizing.

A very useful means of measuring the modification produced by periodic acid is found in the alkaline fluidity as described by R. W. Kerr in: "Chemistry and Industry of Starch" 1944, Academic Press p. 95. The method, as described below, has been used to characterize the starch product oxidized by periodic acid.

#### Alkaline fluidity

Five g. starch, dry weight basis, are wet with 10 ml. of distilled water in a 250-ml. Pyrex beaker. At 25° C., 90 ml. of a 1% solution of NaOH are added with stirring, and the stirring is continued for 3 minutes from the time the sodium hydroxide is poured in. The mixture is allowed to stand 27 min. more at 25° C. At this time the contents are poured into a standardized glass funnel with a special tip and the quantity

of starch solution which runs from the funnel in 70 secs. at 25° C. is noted. This amount, measured in ml., is taken as the fluidity, e. g. the acid-modified thin-boiling starches of commerce with a fluidity of 40 will be fluid enough for 40 ml. of solution to pass the funnel tip in 70 sec., with a fluidity of 60, 60 ml., etc. If 100 ml. water are poured into the standard funnel at 25° C. 100 ml. will be delivered in 70 sec. Relatively, then, water might be said to have a fluidity of 100 ml. by this test.

#### EXAMPLE I

##### Oxidation of raw corn starch with periodic acid in presence of buffer

181. g. raw corn starch (Globe Pearl—moisture content=10.4%) is added to 1468 ml. buffer and stirred vigorously at room temperature with a mechanical stirrer so that the starch does not settle out. The pH of the starch in buffer slurry is 4.72.

181. g. raw corn starch (Globe Pearl—moisture content=10.4%) is added to 1468 ml. buffer and stirred vigorously at room temperature with a mechanical stirrer so that the starch does not settle out. The pH of the starch in buffer slurry is 4.72.

A suitable buffer is made by dissolving 4.5 g. sodium acetate ( $\text{CH}_3\text{COONa} \cdot 3\text{H}_2\text{O}$ —molecular weight =136.09) and 2.0 g. glacial acetic acid ( $\text{CH}_3\text{COOH}$ —molecular weight=60.05) in water and diluting to a final volume of one liter. This gives a solution approximately 0.033 molal in sodium acetate and 0.033 molal in acetic acid. The pH of the buffer solution is 4.7.

In these examples, a volume of buffer solution is taken so that the combined volume of buffer plus that of the added acid is such that the starch concentration is approximately one lb. per gallon of added liquid. This concentration is determined from the weight of the starch "as is" and the moisture content is ignored in calculating the amount of added liquid.

To the starch in buffer slurry is added gradually 40 ml. of a 0.0498 molal solution of periodic acid. Stirring is continued during the addition of acid and for 15 minutes thereafter. At the end of that time the test for periodic acid is negative and the pH of the slurry is 4.70. The slurry is filtered by suction on a Büchner funnel and the filter cake is thoroughly washed with water. The cake is resuspended in water, stirred vigorously for five minutes, and filtered a second time. This operation is repeated a third time. The filter cake is then free of iodic acid and iodates, and has a pH of 5.45.

The filter cake is broken into small pieces and allowed to air-dry for several days. The lumps are broken up by gentle manual grinding with a mortar and pestle and the starch screened through a 200-mesh screen. The product is a fine, white powder resembling starch in appearance. Weight of product is 175 g. with a moisture content of 9.9%.

| Properties                                                                     | Original Starch                                                                   | Oxidized Starch                                                                                                                                                                |
|--------------------------------------------------------------------------------|-----------------------------------------------------------------------------------|--------------------------------------------------------------------------------------------------------------------------------------------------------------------------------|
| Alkaline Fluidity—<br>Film Strength p. s. i                                    | 0.7<br>8,800                                                                      | 70.0<br>7,100 (81% of original film strength).                                                                                                                                 |
| Film Solubility-----                                                           | Films do not dissolve at pH 11.5 and 95°-100° C., but break into large fragments. | At pH 9.6 and above and 80° C. films disintegrate into small fragments which diminish in size as temperature is raised. Practically completely dissolved at pH 9.6 and 100° C. |
| Viscosity 1% Paste: (Aqueous)<br>Setting-up Concentration: (Aqueous), percent. | 21.3 millipoises<br>(mlp.) (pH 5.0).<br>4-4.5                                     | 21.4 mlp. (pH 5.45).<br>5-6 approx.                                                                                                                                            |

7  
EXAMPLE II*Oxidation of Amioca starch with periodic acid in presence of buffer*

181 g. Amioca starch (11.8% moisture) is slurried in 1467 ml. sodium acetate-acetic acid buffer. This is treated at room temperature with a mixture of 20.33 ml. 0.0492 molal periodic acid and 20.33 ml. water, the mixture being adjusted to approximately pH 6.5 with a small amount of sodium bicarbonate. The rest of the procedure is the same as in Example I. The pH of the reaction mixture, measured immediately after the addition of the periodic acid and at the end of the reaction, is 4.7. After 15 minutes there is no positive test for periodic acid, and the starch is filtered from the slurry as in Example I, washed, reslurried, and filtered twice. At the end of this time it is free from iodic acid and iodates. The pH of the filter cake is 5.7. It is allowed to air-dry for several days. Then it is ground as in Example I and screened through a 100-mesh screen.

The product resembles the original Amioca except that it has a somewhat more granular appearance. Its moisture content is 12.9%, and its properties are tabulated below:

| Properties              | Original Starch                   | Oxidized Starch                |
|-------------------------|-----------------------------------|--------------------------------|
| Alkaline Fluidity       | 0.4                               | 38.9                           |
| Film strength, p. s. i. | 5,900                             | 6,300                          |
| Film solubility         | Dissolves at pH 7.5 and 80-85° C. | Dissolves at pH 7.5 and 60° C. |

## EXAMPLE III

*Oxidation of wheat starch with periodic acid in presence of buffer*

185.4 g. commercial wheat starch (12.6% moisture) is slurried in 1488 ml. sodium acetate-acetic acid buffer. To this is added at room temperature 20.33 ml. of 0.0492 molal periodic acid. Measurements of pH are as follows:

- (1) Buffer solution—4.7
- (2) Starch slurry in buffer—4.7
- (3) Starch slurry in buffer after addition of acid—4.69
- (4) Starch slurry in buffer after addition of acid 15 minutes later—4.68

The mixture is stirred mechanically for 15 minutes after addition of the periodic acid. At the end of ten minutes the test for periodic acid is negative, but stirring is continued for 5 minutes more. The product is dewatered as in Example I. It is necessary to filter the starch four times in order to obtain it free from iodic acid. The final pH of the filter cake is 5.35. The starch is allowed to air-dry several days, ground and screened through a 100-mesh screen. The yield of product is 185.5 g. with a moisture content 11.5%.

| Property                | Original Starch                                                              | Oxidized Starch                                                    |
|-------------------------|------------------------------------------------------------------------------|--------------------------------------------------------------------|
| Alkaline Fluidity       | 2.8                                                                          | 53.0                                                               |
| Film strength, p. s. i. | 7,600                                                                        | 7,100                                                              |
| Film solubility         | Does not dissolve but breaks merely into fragments at pH 11.5 and 95-100° C. | Soluble at 95° C. and pH 10.5 and at higher pH's and temperatures. |

## 8

## EXAMPLE IV

*Oxidation of tapioca starch with periodic acid in buffer*

182.4 g. tapioca starch ("Best Maris" grade; 11.2% moisture) is slurried in 1386 ml. sodium acetate-acetic acid buffer at approximately pH 4.5. A mixture of 40.7 ml. 0.0492 molal periodic acid and 81.4 ml. water is adjusted to pH 4.7 with sodium bicarbonate and then added to the starch slurry at room temperature. The mixture is stirred vigorously with a mechanical stirrer. The pH of the mixture immediately after addition of the periodic acid is 4.7 and remains at this value during the reaction.

The mixture is stirred for 15 minutes after the addition of acid. At the end of seven minutes the test for periodic acid is negative, but stirring is continued until the end of the 15-minute period.

20 The product is then dewatered by suction as in the previous examples. After three filtrations the filter cake is found to be free from iodic acid and its final pH is 5.65. The starch is allowed to air-dry for 3 days. It is powdered and screened through a 100-mesh screen. Weight of product obtained is 186.0 g. at 15.3% moisture content.

| Properties              | Original Starch                                 | Oxidized Starch                         |
|-------------------------|-------------------------------------------------|-----------------------------------------|
| Alkaline fluidity       | 2.8                                             | 68.5                                    |
| Film strength, p. s. i. | 9000                                            | 6400                                    |
| Film solubility         | Films do not dissolve at pH 11.5 and 95-100° C. | Films dissolve at pH 7.5 and 75°-80° C. |

## 35

## EXAMPLE V

*Oxidation of corn starch in absence of buffer*

179.4 g. of a crude corn starch (containing 1.23% protein and 9.7% moisture) is slurried in 1486 ml. distilled water and the pH of the mixture adjusted to pH 6.53 with 0.8 ml. 6-normal acetic acid. To this is added at room temperature (24° C.) 22.4 ml. of 0.0447 molal periodic acid. The mixture is stirred for 20 minutes. At the end of this period the test for periodic acid is negative and the pH value has fallen to 6.37. The oxidized starch is recovered by filtration as in the preceding examples. Three filtrations are required to obtain a product free from iodic acid. 45 The pH of the final filter cake is 7.04. The product is allowed to air-dry for several days. Its weight is 192 grams with moisture content 18.0%.

| Properties              | Original Starch                                                           | Oxidized Starch                                                                                                                       |
|-------------------------|---------------------------------------------------------------------------|---------------------------------------------------------------------------------------------------------------------------------------|
| Alkaline fluidity       | 0.3                                                                       | 42.3                                                                                                                                  |
| Film strength, p. s. i. | 4000                                                                      | 3500                                                                                                                                  |
| Film solubility         | Does not dissolve at pH 11.5 and 95-100° C.; breaks into large fragments. | Does not dissolve, but at pH 7.5 and room temperature breaks into fragments which become very small as pH and temperature are raised. |

65 From the foregoing description; it will be seen that the extent to which a starch is modified depends, in part, on the nature of the starch itself and, in part, on the amount of acid used per given weight of starch. The foregoing examples illustrate the preparation of starches having a wide range of modification, as shown by the fact that the alkaline fluidity values varied from 38.9 (Example II) to 70 (Example I). It will be obvious that materials having higher or lower degrees of modification than those given in the ex-

amples can be obtained by varying the amount of acid used for a given amount of starch.

In accordance with the invention, starches are oxidized to provide modified starches having alkaline fluidities by the Kerr method ranging from about 30 to about 90, the products having the most useful properties ranging in alkaline fluidity from about 40 to about 70.

I claim:

1. Oxidized starch dispersible in water to form highly viscous water pastes and slurries at about pH 5 to about pH 7 from which are deposited films having good flexibility and high tensile strength and which are readily dispersible in alkaline solutions, said oxidized starch having an alkaline fluidity ranging from about 30 to about 90, said oxidized starch being prepared by a process comprising reacting starch in an aqueous liquid medium with periodic acid in an amount ranging from about 0.05 part to about 0.5 part by weight for each 100 parts by weight of dry starch, calculated as  $\text{HIO}_4 \cdot 2\text{H}_2\text{O}$ , at a pH of from about 4.5 to about 7.0 at a temperature and for a time sufficient to substantially completely react the periodic acid with the starch.

2. The method of oxidizing starch to increase the alkali solubility thereof which comprises reacting starch in an aqueous liquid medium with periodic acid in an amount ranging from about 0.05 part to about 0.5 part by weight for each 100 parts by weight of dry starch, calculated as  $\text{HIO}_4 \cdot 2\text{H}_2\text{O}$ , at a pH of from about 4.5 to about 7.0 at a temperature and for a time sufficient to substantially completely react the periodic acid with the starch.

3. The method of oxidizing starch to increase the alkali solubility thereof which comprises reacting starch in an aqueous liquid medium with periodic acid in an amount ranging from about 0.1 part to about 0.35 part by weight for each 100

parts by weight of dry starch, calculated as  $\text{HIO}_4 \cdot 2\text{H}_2\text{O}$ , at a pH of from about 4.5 to about 7.0 at a temperature and for a time sufficient to substantially completely react the periodic acid with the starch.

4. The method of oxidizing starch to increase the alkali solubility thereof which comprises reacting starch in an aqueous liquid medium with periodic acid in an amount ranging from about 0.1 part to about 0.35 part by weight for each 100 parts by weight of dry starch, calculated as  $\text{HIO}_4 \cdot 2\text{H}_2\text{O}$ , at a pH of from about 4.5 to about 6.0 at a temperature and for a time sufficient to substantially completely react the periodic acid with the starch.

5. The method of oxidizing starch to increase the alkali solubility thereof which comprises reacting starch in an aqueous liquid medium at a concentration of about 1 lb. of starch per gallon of liquid with periodic acid in an amount ranging from about 0.1 part to about 0.35 part by weight for each 100 parts by weight of dry starch, calculated as  $\text{HIO}_4 \cdot 2\text{H}_2\text{O}$ , at a pH of from about 4.5 to about 6.0 at a temperature of from about 15° C. to about 35° C. and for a time sufficient to substantially completely react the periodic acid with the starch.

WILLIAM E. C. YELLAND.

#### REFERENCES CITED

The following references are of record in the file of this patent:

Chem. Abstracts, vol. 32, page 5280<sup>8</sup>, 1938.

Chem. Abstracts, vol. 32, page 5246<sup>1</sup>, 1938.

Chem. Abstracts, vol. 32, page 825<sup>3</sup>, 1938.

Grangaard et al., Paper Trade Journal, vol. 115,

No. 7, August 13, 1942, pages 41-46.

Carbohydrate Chemistry by Goepp, 1948, pages

40 581 and 582.